

## 1

3,512,982

NUCLEIC ACIDS AS FOG STABILIZERS FOR  
PHOTOGRAPHIC EMULSIONS

Robert C. Taber, William H. Russell, and Charles A. Goffe, Rochester, N.Y., assignors to Eastman Kodak Company, Rochester, N.Y., a corporation of New Jersey  
No Drawing. Filed Apr. 6, 1967, Ser. No. 628,830  
Int. Cl. G03c 5/30, 1/34

U.S. CL. 96—66.5

12 Claims

## ABSTRACT OF THE DISCLOSURE

A photographic silver halide emulsion or photographic element containing a fog-stabilizing amount of a nucleic acid, e.g., ribonucleic acid or deoxyribonucleic acid. Developing photographic elements in the presence of a nucleic acid is also described.

## BACKGROUND OF THE INVENTION

## Field of the invention

This invention relates to new and improved antifoggants and stabilizers for photographic elements and to photographic silver halide emulsions containing said antifoggants and stabilizers therein. The invention also relates to a process of developing photographic elements in the presence of new and improved antifoggants.

## Description of the prior art

During development of a silver halide emulsion, small amounts of silver halide are reduced to metallic silver regardless of whether or not they have been exposed. This reduction of silver ion produces a background fog which is more specifically referred to as chemical fog. This fog is particularly noticeable when the film is given more development than intended either because of longer processing time or higher processing temperature or a combination of both.

Chemical fog, apparent in most silver halide systems, has been reduced by prior art methods of processing exposed silver halide material in the presence of compounds which restrict development of unexposed silver halide. Such compounds can be incorporated in the silver halide emulsion or in the processing solutions for developing such silver halide emulsions. Compounds which have been found to have a chemical fog inhibiting effect on emulsions which have been subjected to high temperature and high humidity conditions are referred to as emulsion stabilizers. On the other hand, compounds which have been found to have chemical fog inhibiting effects on emulsions which have not been exposed to adverse storage conditions are referred to as antifoggants. Although a large number of emulsion stabilizers and antifoggants have been used in the prior art, many of these compounds cause undesirable losses in emulsion speed and contrast and others lack adequate compatibility with emulsion gelatin. Some addenda which have been used in the past to control extended development fog have the disadvantage of attacking the latent image. For example, mercuric chloride added to a photographic emulsion controls fog but results in loss of density if the exposed film is not processed soon after exposure.

## SUMMARY OF THE INVENTION

According to one embodiment of this invention, there is incorporated into the silver halide emulsion of a photographic element or in a layer contiguous to the silver halide emulsion, a fog-stabilizing amount of a nucleic acid. The nucleic acid stabilizes the emulsion against fog when

## 2

the dried emulsion has been subjected to a prolonged high humidity and temperature incubation period without adversely affecting other sensitometric properties.

According to another embodiment of the invention, a photographic element comprising a support coated with at least one silver halide emulsion layer is developed in the presence of a nucleic acid. Preferably, the nucleic acid is present in the photographic element but it may be present elsewhere in the system—e.g., in the developer.

DESCRIPTION OF THE PREFERRED  
EMBODIMENTS

The nucleic acid may be incorporated into the silver halide emulsion of a photographic element or in a layer contiguous to the silver halide emulsion in any amount which will stabilize the silver halide emulsion against fog. In general, a concentration of the nucleic acid in an amount of from about 0.025 to about 10, preferably about 0.050 to about 2, grams per mole of silver in the silver halide emulsion can be used with good results.

Nucleic acids are made up of three components, liberated on acid hydrolysis: an organic base or bases, phosphoric acid and a sugar. As far as is known, the sugar unit is either ribose or 2-deoxyribose. Both deoxyribonucleic acid (DNA) and ribonucleic acid (RNA) contain the bases adenine, guanine and cytosine. In DNA, the fourth base is thymine while in RNA the fourth base is uracil. In our invention, either DNA alone, RNA alone or mixtures of DNA and RNA can be employed.

The preparation of photographic silver halide emulsions such as are suitably stabilized with a nucleic acid typically involves three separate operations: (1) emulsification and digestion of silver halide, (2) the freeing of the emulsion of excess water-soluble salts, suitably by washing with water, and (3) the second digestion or "after-ripening" to obtain increased emulsion speed or sensitivity. (Mees, "The Theory of the Photographic Process," 1954.) The nucleic acid can be added to the emulsion before the final digestion or after-ripening or it can be added immediately prior to the coating.

The silver halide emulsion of a photographic element containing the antifoggants of this invention can contain conventional addenda such as gelatin plasticizers, coating aids, antifoggants such as the azaindines and hardeners such as aldehyde hardeners, e.g., formaldehyde, mucochloric acid, glutaraldehyde bis(sodium bisulfite), maleic dialdehyde, aziridines, dioxane derivatives and oxypolysaccharides. Sensitizing dyes useful in sensitizing such emulsions are described, for example, in U.S. Pats. 2,526,632 of Brooker and White issued Oct. 24, 1950, and 2,503,776 of Sprague issued Apr. 11, 1950. Spectral sensitizers which can be used are the cyanines, merocyanines, complex (trinuclear) cyanines, complex (trinuclear) merocyanines, styryls, and hemicyanines. Developing agents can also be incorporated into the silver halide emulsion if desired or can be contained in a separate underlayer. Various silver salts can be used as the sensitive salt such as silver bromide, silver iodide, silver chloride, or mixed silver halides such as silver chlorobromide or silver bromoiodide.

The silver halide emulsion layer of a photographic element containing the antifoggants of the invention can contain any of the hydrophilic, water-permeable binding materials suitable for this purpose. Suitable materials include gelatin, colloidal albumin, polyvinyl compounds, cellulose derivatives, acrylamide polymers, etc. Mixtures of these binding agents can also be used. The binding agents for the emulsion layer of the photographic element can also contain dispersed polymerized vinyl compounds. Such compounds are disclosed, for example, in U.S. Pats. 3,142,568 of Nottorf issued July 28, 1964; 3,193,386 of White issued July 6, 1965; 3,062,674 of

Houck, Smith and Yudelson issued Nov. 6, 1962; and 3,220,844 of Houck, Smith and Yudelson issued Nov. 30, 1965; and include the water-insoluble polymers of alkyl acrylates and methacrylates, acrylic acid, sulfoalkyl acrylates or methacrylates and the like.

The silver halide emulsion of a photographic element containing the antifoggants of the invention can be coated on a wide variety of supports. Typical supports are cellulose nitrate film, cellulose ester film, polyvinyl acetal film, polystyrene film, poly(ethylene terephthalate) film and related films or resinous materials as well as glass, paper, metal and the like. Supports such as paper which are coated with  $\alpha$ -olefin polymers, particularly polymers of  $\alpha$ -olefins containing two or more carbon atoms, as exemplified by polyethylene, polypropylene, ethylene-butene copolymers and the like can also be employed.

The speed of the photographic emulsions containing the antifoggants of the invention can be further increased by including in the emulsions a variety of hydrophilic colloids such as carboxymethyl protein of the type described in U.S. Pat. 3,011,890 of Gates, Jr., Miller and Koller issued Dec. 5, 1961, and polysaccharides of the type described in Canadian Pat. 635,206 of Koller and Russell issued Jan. 23, 1962.

Photographic emulsions containing the antifoggants of the instant invention can also contain speed-increasing compounds such as quaternary ammonium compounds, polyethylene glycols or thioethers. Frequently, useful effects can be obtained by adding the aforementioned speed-increasing compounds to the photographic developer solutions instead of, or in addition to, the photographic emulsions.

Photographic elements containing the antifoggants of the invention can be used in various kinds of photographic systems. In addition to being useful in X-ray and other non-optically sensitized systems, they can also be used in orthochromatic, panchromatic and infrared sensitive systems. The sensitizing addenda can be added to photographic systems before or after any sensitizing dyes which are used.

Silver halide emulsions containing the antifoggants of the invention can be used in color photography, for example, emulsions containing color-forming couplers or emulsions to be developed by solutions containing couplers or other color-generating materials, emulsions of the mixed-packet type such as described in U.S. Pat. 2,698,794 of Godowsky issued Jan. 4, 1955; in silver dye-bleach systems; and emulsions of the mixed-grain type such as described in U.S. Pat. 2,592,243 of Carroll and Henson issued Apr. 8, 1952.

Silver halide emulsions containing the antifoggants of the invention can be sensitized using any of the well-known techniques in emulsion making, for example, by

halide emulsion layer. Such processes are described in U.S. Pats. 2,352,014 of Rott issued June 20, 1944; 2,543,181 of Land issued Feb. 27, 1951; and 3,020,155 of Yackel, Yutzy, Foster and Rasch issued Feb. 6, 1962. The emulsions can also be used in diffusion transfer color processes which utilize a diffusion transfer of an image-wise distribution of developer, coupler or dye, from a light-sensitive layer to a second layer, while the two layers are in close proximity to one another.

While it is preferred to utilize the antifoggants of the invention by incorporating them directly into a photographic element, the antifoggants could also be utilized by incorporating them into a photographic developer, since image formation would still take place in the presence of the antifoggants and they would still perform their antifoggant function.

The antifogging agents of this invention can be incorporated to advantage during manufacture in silver halide emulsions representing the variations described above. Moreover, fog control in binderless silver halide films prepared by vapor deposition of silver halide on a suitable support can be achieved by coating the antifogging agents of the invention over the vapor deposited layer of silver halide.

The invention can be further illustrated by the following examples or preferred embodiments thereof; although it will be understood that these examples are included merely for purposes of illustration and are not intended to limit the scope of the invention.

#### EXAMPLE 1

Separate samples of a silver chlorobromide emulsion containing, respectively, no antifogging,  $HgCl_2$  and varying amounts of RNA are ripened to optimum sensitivity and coated on a cellulose acetate film support at a coverage of 478 milligrams of silver per square foot and 474 milligrams of gelatin per square foot. One set of film coatings is exposed for  $10^{-6}$  second on an intensity scale sensitometer, processed for three minutes in Kodak D-19 Developer containing 10 milligrams of potassium iodide per liter, fixed, washed and dried. The procedure is repeated with a second set of film coatings except that the film coating is processed for eight minutes in the developer. A third set of film coatings exposed three days earlier and kept at 78° F. is processed for three minutes in the developer, fixed, washed and dried. The photographic results obtained from these tests are set forth in Table I. In this table,  $D_1$  is the loss in density of film coatings which have been kept at 78° F. for three days after an exposure which produces a fresh density of 1.0; and  $D_2$  is the loss in density of film coatings which have been kept at 78° F. for three days after an exposure which produces a fresh density of 2.0.

TABLE I

| Compound | Conc. in<br>mg./mole | 3 minute processing |            | 8 minute<br>processing |      | $D_1$ | $D_2$ |
|----------|----------------------|---------------------|------------|------------------------|------|-------|-------|
|          |                      | Ag                  | Rel. speed | Gamma                  | Fog  |       |       |
| Control  |                      | 214                 |            | 4.30                   | 0.22 | 0.74  | 0.12  |
| $HgCl_2$ | 0.14                 | 180                 |            | 4.30                   | 0.08 | 0.10  | 0.24  |
| RNA      | 300                  | 198                 |            | 4.10                   | 0.08 | 0.35  | 0.12  |
| RNA      | 350                  | 190                 |            | 3.90                   | 0.06 | 0.24  | 0.14  |
| RNA      | 375                  | 186                 |            | 3.76                   | 0.06 | 0.21  | 0.06  |
| RNA      | 400                  | 182                 |            | 3.44                   | 0.04 | 0.20  | 0.10  |
| RNA      | 425                  | 178                 |            | 3.44                   | 0.04 | 0.19  | 0.05  |

digesting with naturally active gelatin or various sulfur, selenium, tellurium compounds and/or gold compounds. The emulsions can also be sensitized with salts of noble metals of Group VIII of the Periodic Table which have an atomic weight greater than 100.

Silver halide emulsions containing the antifoggants of the invention can be used in diffusion transfer processes which utilize the undeveloped silver halide in non-image areas of the negative to form a positive by dissolving the undeveloped silver halide and precipitating it on a silver receiving layer in close proximity to the original silver

70  
75

The results in the above table show that RNA compares favorably with  $HgCl_2$  in its ability to control extended development fog that it shows less tendency to attack the latent image as evidenced by the resistance to density loss ( $D_1$  and  $D_2$ ) for RNA as compared to the mercuric chloride salt.

#### EXAMPLE 2

This example illustrates the use of RNA as an antifogging agent in a high speed silver halide emulsion of the type used in medical X-ray films. Two silver bromoiodide

emulsions, one containing no antifogging agent and the other containing RNA, are coated on a polyethylene terephthalate film support at a coverage of 454 milligrams of silver per square foot and 504 milligrams of gelatin per square foot. The coatings are given a  $\frac{1}{20}$  second simulated blue screen exposure and processed for six minutes in Kodak D-19 Developer containing 10 milligrams of potassium iodide per liter. A second set of coatings, which have been incubated for two weeks at 120° F. and 50 percent relative humidity, are processed in the same manner. The photographic results obtained from these tests are set forth in Table II.

TABLE II

| Compound     | Cone. in<br>mg./mole | Fresh |                   | 2 week incubation<br>at 120° F. and 50%<br>relative humidity |                   |
|--------------|----------------------|-------|-------------------|--------------------------------------------------------------|-------------------|
|              |                      | Ag    | Relative<br>speed | Fog                                                          | Relative<br>speed |
| Control..... | 100                  | 100   | 0.15              | 95                                                           | 0.59              |
| RNA.....     | 100                  | 100   | 0.15              | 100                                                          | 0.32              |

The results in Table II show that RNA controls incubation fog without adversely affecting sensitometric properties.

## EXAMPLE 3

A silver bromoiodide emulsion is prepared corresponding to Emulsion No. 12 described in "Empirical Relations Between Sensitometric and Size-Frequency Characteristics in Photographic Emulsion Series" by Trivelli and Smith, Photo. Journal, May 1939, page 330. Two samples of this emulsion, one (the control) containing no antifogging agent and the other containing 1.0 gram of RNA per mole of silver, are coated on a cellulose acetate film support at a coverage of 450 milligrams of silver and 1030 milligrams of gelatin per square foot. A sample of each film coating is exposed for  $\frac{1}{25}$  second on an intensity scale sensitometer, processed for five minutes in Kodak Developer DK-50, fixed, washed and dried. The photographic results obtained are listed in Table III.

TABLE III

| Antifogging  | Relative<br>speed | Gamma | Fog  |
|--------------|-------------------|-------|------|
| Control..... | 100               | 0.96  | 0.12 |
| RNA.....     | 151               | 0.97  | 0.10 |

The results in Table III show that RNA gives antifogging action and allows chemical sensitization to a higher speed.

Although the invention has been described in considerable detail with reference to certain preferred embodiments thereof, it will be understood that variations and modifications can be effected without departing from the

spirit and scope of the invention as described hereinabove and as defined in the appended claims.

We claim:

1. A composition comprising a photographic silver halide emulsion containing a fog-stabilizing amount of "ribonucleic acid" or "deoxyribonucleic acid."
2. The composition of claim 1 wherein said nucleic acid, "ribonucleic acid" or "deoxyribonucleic acid," is present in an amount of from about 0.025 to about 10 grams per mole of silver in said silver halide emulsion.
3. A photographic element comprising a support coated with a silver halide layer, said element containing a fog-stabilizing amount of "ribonucleic acid" or "deoxyribonucleic acid."
4. The photographic element of claim 3 wherein said layer is a silver halide emulsion.
5. The photographic element of claim 4 wherein said nucleic acid, "ribonucleic acid" or "deoxyribonucleic acid," is present in an amount of from about 0.025 to about 10 grams per mole of silver in said silver halide emulsion.
6. The photographic element of claim 4 wherein said nucleic acid, "ribonucleic acid" or "deoxyribonucleic acid," is present in said silver halide emulsion.
7. The photographic element of claim 4 wherein said nucleic acid is present in a layer contiguous to said silver halide emulsion.
8. The photographic element of claim 7 wherein said "ribonucleic acid or deoxyribonucleic acid" is present in said silver halide emulsion.
9. In a process of developing a photographic element comprising a support coated with at least one silver halide emulsion layer, the improvement comprising developing said photographic element in the presence of a "stabilizing amount of ribonucleic acid or deoxyribonucleic acid."
10. The composition of claim 1 containing a fog-stabilizing amount of ribonucleic acid.
11. The photographic element of claim 3 containing a fog-stabilizing amount of ribonucleic acid.
12. The process of claim 9 in which the improvement comprises developing said element in the presence of ribonucleic acid.

## References Cited

## UNITED STATES PATENTS

- 3,023,103 2/1962 Dersch et al. .... 96—109  
3,148,066 9/1964 Holstead .... 96—109

NORMAN G. TORCHIN, Primary Examiner

R. E. FICHTER, Assistant Examiner

U.S. Cl. X.R.

96—109

#### **Disclaimer**

3,512,982.—*Robert C. Taber, William H. Russell, and Charles A. Goffe*, Rochester, N.Y. NUCLEIC ACIDS AS FOG STABILIZERS FOR PHOTOGRAPHIC EMULSIONS. Patent dated May 19, 1970. Disclaimer filed Apr. 5, 1971, by the assignee, *Eastman Kodak Company*.

Hereby enters this disclaimer to claims 1 through 12, inclusive.  
[Official Gazette June 29, 1971.]